

Feb. 17, 1931.

H. M. COX ET AL

1,792,573

METHOD OF HEAT TREATING IRON AND STEEL SHEETS

Filed Jan. 31, 1929



Inventor

Herbert M. Cox  
Cary M. Smith

William J. O'Brien  
Attorney

## UNITED STATES PATENT OFFICE

HERBERT M. COX, OF CANTON, AND CARY M. SMITH, OF MASSILLON, OHIO, ASSIGNEES,  
BY MESNE ASSIGNMENTS, TO REPUBLIC STEEL CORPORATION, OF YOUNGSTOWN,  
OHIO, A CORPORATION OF NEW JERSEY

## METHOD OF HEAT TREATING IRON AND STEEL SHEETS

Application filed January 31, 1929. Serial No. 336,497.

This invention relates in general to the manufacture of iron and steel sheets, and more particularly to the heat treatment or normalizing of such sheets for the purpose of developing certain desirable physical and mechanical properties therein.

As is well known, a sheet which has been normalized under the ordinary practice of normalizing, as for example in an open annealing furnace, has better drawing and stamping qualities than a box-annealed sheet, but owing to its stiffness, is likely to wrinkle in forming, and its adaptation for difficult drawing and stamping operations has therefore been somewhat limited.

A box-annealed sheet, on the other hand, has the required degree of softness, but when subjected to difficult drawing and stamping operations, is likely to break or tear.

In recent years, a demand has arisen, particularly in the automobile industry, for a sheet in which is combined the drawing and stamping qualities of a normalized sheet with the softness obtainable in a box-annealed sheet, and it is a primary object of the present invention to provide a method of imparting to low-carbon steel sheets certain qualities as to hardness and structure, which will enable these sheets to be subjected to deep drawing, stamping and other severe forming operations, without danger of wrinkling, breaking, tearing or cracking.

In accordance with the invention, low-carbon sheets of steel, as produced by ordinary hot rolling methods, are first subjected to a preheating treatment, the object of which is to promote grain growth in the metal and to promote spheroidization of the carbides present in the steel so as to decrease their hardening effect on the final product. This preheating or annealing treatment is preferably carried on at a temperature near the lower critical point of the metal, and for a sufficient length of time to produce the aforementioned effects.

The sheets are then heated to a maximum temperature somewhat above the upper critical point of the metal, and are retained at this temperature for a sufficient length of time to cause a rearrangement in the grain structure

and solution of the carbides present for the purpose of destroying the strains and banded conditions which have been induced in the sheets as a result of the hot rolling operations.

Following this treatment, the sheets are quickly cooled to a temperature near or below the lower critical point of the metal, the effect of this treatment being to produce a small grain structure in the metal of the type desired in the finished product.

The sheets are then reheated to a temperature near or slightly above the lower critical point of the metal, and are retained at this temperature for a sufficient length of time to induce a maximum degree of softness in the sheets. Following this treatment, the sheets are allowed to cool slowly and are discharged from the furnace at a temperature not in excess of 1100° F.

## Example

As an example of the above described heat treatment, attention is directed to the curve shown in the accompanying drawing, forming a part of this specification, and showing the cycle of treatment as applied to hot rolled 22-gauge, open steel sheets, having a carbon content varying from .07% to .12%.

The sheets were conveyed on rolls through a continuous open annealing furnace, approximately 200 feet long, and divided into a number of zones of different temperatures.

In the first or preheating zone, the sheets were rapidly heated to a temperature of 1325° F., and retained at this temperature for approximately three minutes. The effects of this treatment were a marked grain growth in the metal, and spheroidization of the carbides present.

The sheets were then heated to a temperature of 1800° F., and retained at this temperature for approximately three minutes. The effects of this treatment were a rearrangement in the grain structure, solution of the carbides present and a destruction of the strains and banded conditions which had been induced in the sheets as a result of the hot rolling operations which they had undergone.

Following this treatment, the sheets were

55

60

65

70

75

80

85

90

95

100

rapidly cooled to a temperature of 1100° F., and retained at this temperature for about one minute in order to insure that all parts of the sheet were at the same temperature.

6 The effect of this rapid cooling was the production of a small grain structure of the desired type in the finished sheets.

The sheets were then reheated to a temperature of 1375° F., and retained at this temperature for about four minutes. This final treatment induced a maximum degree of softness in the sheets. The sheets were permitted to cool slowly and were discharged from the furnace at a temperature of about 1000° F.

15 The sheets, thus treated, were then subjected to a series of physical and mechanical tests, and were found to have a degree of softness and stiffness, which made them admirably adapted for the difficult deep drawing 20 and stamping operations frequently encountered in the manufacture of automobile bodies and the like.

By low carbon iron and steel sheets, as herein described, it is intended to include iron 25 and steel containing up to about .20% carbon, as well as iron and steel containing up to about .20% carbon and in addition small proportions of alloying ingredients, such as copper, molybdenum, etc.

30 As the gauges of sheets vary to a considerable extent, the conditions under which they are hot rolled will vary to some extent, and the strains, banded conditions, grain structure, etc. will likewise vary in accordance 35 with the conditions under which the sheets have been rolled. In addition, the upper critical or  $Ac_3$  point of low carbon steels varies from approximately 1650° F. for steel containing .05% carbon to approximately 46 1550° F. for steel containing .20% carbon. All of these conditions may necessitate a variation in the temperatures employed for the various steps of the heat treatment, as well as a variation in the time required for each 45 step of the treatment. In order to practice these variations it may be necessary to employ a longer furnace than the one above described.

The temperature of the preheating treatment may vary from 1250° F. to 1400° F., and the time of treatment in this temperature range may vary from about one-half to six minutes.

50 The temperature of maximum heating need be but slightly above the upper critical point 55 of the metal. A temperature of 1800° F. has been found to be suitable under most conditions, but the temperature may vary from 1600° F. to 1800° F. without departing from the scope of the invention. The time of treatment at the maximum temperature may likewise vary from two to six minutes.

55 The rapid cooling of the sheets from the maximum temperature may proceed to any temperature near or below the lower critical 60 point of the metal, but in practice the lowest

temperature may vary from 1200° F. to 1100° F. Owing to the necessity of reheating the sheets, they need be maintained at this low temperature only momentarily, but in practice, in order to insure all parts of the sheet being at a uniform temperature, it is desirable to maintain the sheets at this temperature for about a minute. Here again, however, there may be a variation from a small fraction of a minute up to about two minutes.

70 In reheating the sheets, the temperature to which they are reheated may vary from 1250° F. to 1400° F., and the time of treatment in this temperature range may vary from two to eight minutes.

75 Following the reheating treatment, the sheets may be slowly cooled and discharged from the furnace into the atmosphere at a temperature not in excess of 1100° F.

80 Having described our invention, and in what manner the same is to be practiced, we claim:

1. The method of heat treating iron and steel sheets which comprises heating the sheets to a temperature within the range 90 1250° F.-1400° F., maintaining the sheets at this temperature for a period varying from about one-half to six minutes, then heating the sheets to a temperature within the range 95 1600° F.-1800° F., maintaining the sheets at 100 said temperature for a period varying from two to six minutes, then cooling the sheets rapidly to a temperature within the range 1200° F.-1100° F., maintaining the sheets at this temperature for a period varying from a small fraction of a minute to two minutes, then reheating the sheets to a temperature within the range 105 1250° F.-1400° F., maintaining the sheets at this temperature for a period varying from two to eight minutes, and then permitting the sheets to cool to 110 atmospheric temperature.

2. The method of heat treating iron and steel sheets which comprises heating the sheets to a temperature of about 1325° F., 110 maintaining the sheets at this temperature for about three minutes, then heating the sheets to a temperature of about 1800° F., maintaining the sheets at this temperature for about three minutes, then cooling the sheets rapidly to a temperature of about 115 1100° F., maintaining the sheets at this temperature for about one minute, then reheating the sheets to a temperature of about 1375° F., maintaining the sheets at this temperature for about four minutes, and then permitting the sheets to cool to atmospheric temperature.

3. The method of heat treating iron and steel sheets which comprises heating the sheets to a temperature near the lower critical point of the metal, maintaining the sheets at this temperature for a period varying from about one-half to six minutes, then heating the sheets to a temperature above the upper critical point of the metal, maintaining the 120 125

sheets at this temperature for a period varying from two to six minutes, then cooling the sheets rapidly to a temperature below the lower critical point of the metal, maintaining the sheets at this temperature for a period varying from a small fraction of a minute to two minutes, then reheating the sheets to a temperature near the lower critical point of the metal, maintaining the sheets at this 10 temperature for a period varying from 2 to 8 minutes and then permitting the sheets to cool to atmospheric temperature.

In testimony whereof we affix our signatures.

15 HERBERT M. COX,  
CARY M. SMITH.

20

25

30

35

40

45

50

55

60

65